

## UNITED STATES PATENT OFFICE

2,479,110

PROCESS OF REFORMING A GASOLINE  
WITH AN ALUMINA-PLATINUM-HALO-  
GEN CATALYSTVladimir Haensel, Clarendon Hills, Ill., assignor  
to Universal Oil Products Company, Chicago,  
Ill., a corporation of DelawareNo Drawing. Application November 28, 1947,  
Serial No. 788,673

19 Claims. (Cl. 196—56)

1

This invention relates to a reforming process and more particularly to a process for the reforming of a saturated gasoline fraction in the presence of a particular catalyst and under selected conditions of operation.

The saturated gasoline fraction to be treated in accordance with the present invention comprises straight run gasoline, natural gasoline, etc. The gasoline fraction may be a full boiling range gasoline having an initial boiling point within the range of about 50° to about 100° F. and an end boiling point within the range of about 375° to about 425° F., or it may be a selected fraction thereof which usually will be a higher boiling fraction, commonly referred to as naphtha, and generally having an initial boiling point of from about 150° to about 250° F. and an end boiling point within the range of about 350° to about 425° F.

The term "reforming" is well known in the petroleum industry and refers to the treatment of gasoline fractions to improve the antiknock characteristics. Straight run gasolines contain naphthenic hydrocarbons, particularly cyclohexane compounds, and paraffinic hydrocarbons which usually are of straight chain or slightly branched chain structure, as well as varying proportions of aromatic hydrocarbons. In order to obtain best results in reforming operations it is desired to dehydrogenate the naphthenic hydrocarbons to produce aromatics, to cyclize the straight chain paraffinic hydrocarbons to form aromatics, as well as to effect a controlled type of cracking which is selective both in quality and in quantity. In addition various other concomitant reactions occur such as isomerization, hydrogen transfer, etc.

The cracking or splitting of carbon to carbon bonds is one of the important factors in a successful reforming process. Controlled or selective cracking is highly desirable since such cracking will result in a product of improved antiknock characteristics. In general, the lower molecular weight products have higher octane numbers, and thus a final gasoline product of lower average molecular weight will usually have a higher octane rating. Further, during the cracking reaction, isomerization or other molecular rearrangement occurs which also results in products having higher antiknock characteristics. The selective cracking is also of particular advantage when the charging stock contains component boiling above about 400° F. in order to convert these components to fraction boiling below about 400° F. It is thus seen that the selective cracking results not only in an improved quality product but also in an increase in quantity of the desired products.

2

However, the cracking must be selective and must not result in the decomposition of the normally liquid hydrocarbons substantially or completely into normally gaseous hydrocarbons. The desired selective cracking generally comprises the splitting of a higher boiling hydrocarbon molecule into two molecules both of which are normally liquid hydrocarbons. To a lesser extent it comprises the removal of methyl, ethyl and, to a still lesser extent, propyl groups, in the form of methane, ethane and propane. However, the removal of these radicals is controlled so that not more than one or possibly two of such radicals are removed from a given molecule. For example, decane may be reduced to two pentane molecules, heptane to hexane, nonane to octane or heptane, etc. On the other hand uncontrolled or non-selective cracking will result in the decomposition of normally liquid hydrocarbons into normally gaseous hydrocarbons as, for example, by the continued demethylation of normal heptane to produce 7 molecules of methane.

Another important objection to non-selective or uncontrolled cracking is that this type of cracking will result in the more rapid formation of larger quantities of coke or carbonaceous material which deposits on the catalyst and decreases or destroys its activity to catalyze the desired reactions. This in turn results in shorter processing cycles or periods, with the necessity of more frequent regeneration of the catalyst by burning the carbonaceous products therefrom or, should the catalyst activity be destroyed, it will be necessary to shut down the unit to remove the old catalyst and replace it with new catalyst.

Another important feature in successful reforming processes is the matter of hydrogen production and consumption. Investigation has shown that the presence of hydrogen in the reforming zone further tends to decrease the amount of carbonaceous deposits on the catalyst. Reforming processes effected in the presence of hydrogen are known as "Hydroforming." In view of the fact that the cost of hydrogen is quite high, it is essential that there be no net consumption of hydrogen or, in other words, at least as much hydrogen must be produced in the process as is consumed therein.

In a broad aspect the present invention relates to a process for reforming a gasoline fraction which comprises subjecting said fraction to contact at reforming conditions with a catalyst comprising alumina, platinum and halogen ions.

In a specific embodiment the present invention relates to a process for reforming a straight run gasoline fraction which comprises subjecting said gasoline fraction to contact at a temperature of from about 600° to about 1000° F., a pressure of

from about 50 to about 1000 pounds per square inch and at a weight hourly space velocity of from about 0.5 to about 10, in the presence of from about 0.5 to about 10 mols of hydrogen, with a catalyst comprising alumina, platinum in an amount of from about 0.01% to about 1% by weight of said catalyst, and halogen ions in an amount of from about 0.1% to about 8% by weight of said catalyst.

The use of platinum as a catalyst for conversion processes has been of limited commercial acceptance because of the high cost of the catalyst. The present invention is based on the discovery that exceptionally good catalysts may be prepared to contain very low concentrations of platinum. While these catalysts may contain larger concentrations of platinum, which may range up to about 10% by weight or more of the alumina, it has been found that exceptionally good catalysts may be prepared to contain as low as from about 0.01% to about 1% by weight of platinum. Catalysts of these low platinum concentrations are particularly preferred in the present invention because of the considerably lower cost of the catalyst. It is well known that platinum is very expensive and any satisfactory method of reducing the amount of platinum required in catalysts considerably reduces the cost of the catalyst and thus enhances the attractiveness of the catalyst for use in commercial processes. The platinum generally comprises a major portion of the cost of the catalyst and, therefore, by reducing the amount of platinum required to one half, for example, reduces the cost of the catalyst substantially by one half. Further, for example, when the amount of platinum is reduced to about 0.1% by weight as against 5% by weight, or more, as heretofore required, it is readily apparent that the cost of the catalyst is reduced by at least 50 times.

However, in order to obtain improved results with these low platinum concentrations, it is necessary that a particular type of supporting component must be composited with the platinum. It has been found that alumina shows unexpected advantages for use as a supporting component for the low platinum concentrations, apparently due to some peculiar association of the alumina with the platinum, either as a chemical combination or merely as a physical association. It has been found that the specific combination of alumina and low platinum concentration, not only to be a very active catalyst, but also to have a long catalyst life; that is, the catalyst retains its high activity for long periods of service. After these long periods of service, the catalyst may show a drop in activity and it has further been found that the particular combination of alumina and platinum renders the catalyst susceptible to ready regeneration.

To further improve these catalysts, it is an essential feature of the present invention that the final catalyst contains halogen ions in a specific concentration. It has been found, and will be shown in the following examples, that the presence of halogen ions within a specific range enhances the initial activity of the catalyst and also serves to increase the life of the catalyst. It is believed that the halogen enters into some chemical combination or loose complex with the alumina and/or platinum, and thereby serves to improve the final catalyst.

While any of the halogen ions will serve to effect improved results, the fluoride ions are particularly preferred. Next in order are the chlo-

ride ions, while the bromide and iodide ions are generally less preferred. It is understood that, while all of these halogens will serve to effect an improvement, they are not necessarily equivalent.

The catalyst of the present invention may be prepared in any suitable manner, a particularly preferred method is to prepare alumina by adding a suitable reagent, such as ammonium hydroxide, ammonium carbonate, etc. to a salt of aluminum, such as aluminum chloride, aluminum sulfate, aluminum nitrate, etc. in an amount to form aluminum hydroxide which upon drying is converted to alumina and, in the interest of simplicity, the aluminum hydroxide is referred to as alumina in the present specification and claims in order that the percentages are based on the alumina free of combined water. It has been found that aluminum chloride is generally preferred as the aluminum salt, not only for convenience in subsequent washing and filtering procedures, but also because it appears to give best results.

After the alumina has been formed, it is generally washed to remove soluble impurities. Usual washing procedures comprise washing with water, either in combination with filtration or as separate steps. It has been found that filtration of the alumina is improved when the wash water includes a small amount of ammonium hydroxide. The severity of washing will depend upon the particular method employed in preparing the catalyst. In one embodiment of the invention, the alumina is thoroughly washed with a suitable amount of water and preferably water containing ammonium hydroxide to reduce the chlorine content of the alumina to below about 0.1%. In another embodiment of the invention this washing may be selective to retain chloride ions in an amount of from about 0.2% to about 5% by weight of the alumina on a dry basis. In accordance with this method of preparing the catalyst, the chloride ions are obtained from the original aluminum chloride and are retained in the alumina, thus avoiding the necessity of adding the halogen ions in a later step of catalyst preparation. However, it generally is difficult to control the washing procedure to retain the desired amount of halogen ion and, for this reason, it usually is preferred to wash the alumina to remove substantially all of the chlorine ions and thereafter add the halogen ions in a controlled amount. The addition of the halogen ions in this manner permits better control of the amount of halogen being added. In another embodiment of the invention, the washing may be selective to retain the chloride ions in an amount constituting a portion of the total halogen desired, and the remaining portion of the halogen is then added in a subsequent step. In this method, the halogen ion may comprise the same halogen or a mixture of two different halogens, as for example, chlorine and fluorine.

In some cases, it may be desired to commingle an organic acid and particularly acetic acid which has been found to have a favorable effect on the catalyst. The acetic acid apparently serves to peptize the alumina and thereby renders it in a better condition for compositing with the platinum, and also partly to fix the platinum on the alumina so that migration of the platinum during subsequent heating is minimized. The amount of acetic acid, when employed, will generally be within the range of from about 0.05 to about 0.5 mol of acetic acid per mol of alumina.

Alumina prepared in the above manner, after washing and filtration, is generally recovered as a wet cake. The wet cake is usually made into a slurry with water and sent to a separate zone for further handling. When the halogen ion is to be added separately, it preferably is done at this stage of the catalyst preparation, that is, before the platinum is commingled with the alumina. The halogen ion may be added in any suitable manner. However, the halogen must be added in a form which will readily react with the alumina in order to obtain the desired results and also must not leave undesired deposits in the catalyst. A preferred method of adding the halogen is in the form of an acid, such as hydrogen fluoride, hydrogen chloride, hydrogen bromide and/or hydrogen iodide. Hydrogen fluoride is preferably added as an aqueous solution for ease in handling and for control of the specific amount to be added. Another satisfactory source to be used for adding the halogen is the volatile salts, such as ammonium fluoride, ammonium chloride, etc. The ammonium ions will be removed during the subsequent heating of the catalyst and, therefore, will not leave undesirable deposits in the catalyst. In still another method, the halogen may be added as fluorine, chlorine, bromine, or iodine but, in view of the fact that fluorine and chlorine normally exist as a gas, it is generally preferable to utilize them in the form of a solution for ease in handling. In some cases, the inclusion of certain components will not be harmful but may be beneficial, and in these cases the halogen may be added in the form of salts such as potassium fluoride, sodium fluoride, thorium fluoride, sodium chloride, potassium chloride, etc.

The concentration of halogen ion in the finished catalyst will be within the range of from about 0.1% to about 8% by weight of the alumina on a dry basis. The fluoride ion appears to be more active and therefore will be used within the range of from about 0.1% to about 3% by weight of the alumina on a dry basis. The chloride ion will be used within the range of from about 0.2% to about 8% and preferably from about 0.5% to about 5% by weight of the alumina on a dry basis. It has been found that halogen concentrations below these lower limits do not give the desired improvement and, on the other hand, concentrations of halogen above the upper limits adversely affect the selectivity of the catalyst, thus catalyzing side reactions to an extent greater than desired.

After the alumina and halogen have been intimately mixed, the platinum may be added in any suitable manner. A particularly preferred method is to form a separate solution of chloroplatinic acid in water and introduce hydrogen sulfide into this solution at room temperature, until the chloroplatinic acid solution reaches a constant coloration; that is, will not change color upon the addition of more hydrogen sulfide. The chloroplatinic acid solution is normally light yellow and, upon the addition of hydrogen sulfide gas, turns to a dark brown color. Apparently the chloroplatinic acid and hydrogen sulfide react to form one or more complex chemical compounds. Best results have been obtained in this method when the hydrogen sulfide is added at room temperature to the chloroplatinic acid solution. The addition of hydrogen sulfide at an elevated temperature of 175° F. appears to produce less satisfactory catalysts. The

brown solution of chloroplatinic acid and hydrogen sulfide may then be commingled with the slurry of wet alumina gel at room temperature, and the slurry sufficiently stirred to obtain intimate mixing of the two solutions.

In the preferred embodiment of the invention the platinum is added in an amount to produce a final catalyst containing from about 0.01% to about 1% by weight of platinum.

In another method of operation, chloroplatinic acid solution may be added to the slurry of alumina gel, and hydrogen sulfide then is added to the mixture. In this method of operation it has been found that the hydrogen sulfide may be added at room temperature or at an elevated temperature of 175° F.

In some cases, satisfactory catalysts may be produced by commingling the chloroplatinic acid solution with the slurry of alumina gel, and then drying and heating in the manner to be herein-after set forth. In this method, hydrogen sulfide is not used. However, experiments have shown that the hydrogen sulfide addition is preferable because it tends to further fix the platinum in the form of an insoluble compound on the alumina so that the platinum compounds will not migrate during the subsequent heating of the catalyst.

It has been found that best results are obtained when the platinum is composited with the alumina before the alumina is subjected to substantial heating. As will be shown in the following examples, a higher octane product was obtained when the chloroplatinic acid was added to the wet alumina gel as compared to adding the chloroplatinic acid to alumina which had previously been dried and formed into pills.

After the platinum in proper concentration has been commingled with the alumina, the mixture is preferably dried at a temperature of from about 200 to about 400° F. for a period of from about 4 to 24 hours or more to form a cake. In some cases it is desired to prepare the catalyst in the form of pills of uniform size and shape, and this may readily be accomplished by grinding the partially dried catalyst cake, adding a suitable lubricant, such as stearic acid, rosin, hydrogenated coconut oil, graphite, etc., and then forming into pills in any suitable pelleting apparatus. Particular satisfactory pills comprise those of a size ranging from about  $\frac{1}{8}'' \times \frac{1}{8}''$  to  $\frac{1}{4}'' \times \frac{1}{4}''$  or therabouts. Pills of uniform size and shape may also be formed by extrusion methods. In some cases it may be desired to utilize the catalyst as powder or granules of irregular size and shape, in which cases the pilling and extrusion operations may be omitted.

The catalyst may now be subjected to high temperature treatment, and this may comprise one of several methods. Preferred method is to subject the catalyst to calcination at a temperature of from about 800° to about 1200° F. for a period of from about 2 to 8 hours or more. Another method is to subject the catalyst to reduction with hydrogen or hydrogen-containing gas at a temperature of from about 300° to about 600° F. for about 4 to 12 hours or more, preferably followed by calcination at a temperature of from about 800° to about 1200° F. In still another method the catalyst may be subjected to reduction with hydrogen or hydrogen-containing gas at a temperature of from about 800° to about 1200° F. for a period of from about 2 to 10 hours or more.

In some cases the lubricant will be removed

during the high temperature heating. In other cases as, for example, when graphite is used as the lubricant, the separate high temperature heating step may be omitted, and the effective heat treatment of the catalyst may be obtained in the plant before or during processing of the hydrocarbons.

Although the catalyst of the present invention will have a long life, it may be necessary to regenerate the catalyst after long periods of service. The regeneration may be effected by treatment with air or other oxygen-containing gas to burn carbonaceous deposits therefrom. In general, it is preferred to control the regeneration temperature not to exceed about 1200° F. In some cases it may be desirable to follow the burning operation with treatment with hydrogen-containing gas at temperatures of from about 700° to about 1100° F.

The reforming process will be effected at a temperature within the range of from about 600° to about 1000° F., a pressure within the range of from about 50 to about 1000 pounds per square inch and at a weight hourly space velocity of from about 0.5 to about 10. The weight hourly space velocity is defined as the weight of oil per hour per weight of catalyst in the reaction zone.

Hydrocracking reactions are favored at temperatures within the range of from about 600° to about 700° F. and at pressures within the range of from about 500 to about 1000 pounds or more. Hydrocracking is defined as cracking or splitting of carbon to carbon bonds accompanied by saturation of the fragments so formed by hydrogen present in the reaction zone and, in accordance with the present invention, the hydrocracking will be selective both in quality and in quantity as hereinbefore set forth. On the other hand the aromatization reactions are favored at temperatures within the range of from about 650° to 1000° F. and at lower pressures within the range of from about 50 pounds to about 400 pounds per square inch. It is an essential feature of the present invention that the temperature, pressure and space velocity are correlated to produce the desired aromatization and selective hydrocracking. The exact temperature, pressure and space velocity to be used in any given operation will depend upon the particular gasoline fraction being treated and the particular products desired.

In one embodiment of the process, sufficient hydrogen will be produced in the reforming reaction to furnish the hydrogen required in the process and, therefore, it may be unnecessary to either introduce hydrogen from an extraneous source or to recycle hydrogen within the process. However, it usually will be preferred to introduce hydrogen from an extraneous source, generally at the beginning of the operation, and to recycle hydrogen within the process in order to be assured of a sufficient hydrogen atmosphere in the reaction zone. In some cases the gas to be recycled will contain hydrogen sulfide, introduced with the charge or liberated from the catalyst, and it is within the scope of the present invention to treat the hydrogen containing gas to remove hydrogen sulfide or other impurities before recycling the hydrogen within the process.

The process of the present invention may be effected in any suitable equipment. A particularly suitable process comprises the well known fixed bed system in which the catalyst is disposed in a reaction zone and the hydrocarbons to be treated are passed therethrough in either

upward or downward flow. The products are fractionated to separate hydrogen and to recover the desired products. As hereinbefore set forth, the hydrogen may be recycled for further use in the process. Other suitable units in which the process may be effected include the fluidized type process in which the hydrocarbons and catalysts are maintained in a state of turbulence under hindered settling conditions in a reaction zone, the compact moving bed type in which the catalyst and hydrocarbons are passed either concurrently or countercurrently to each other, and the suspensoid type of operation in which the catalyst is carried into a reaction zone as a slurry in the hydrocarbon oil.

The following examples are introduced to further illustrate the novelty and utility of the present invention, but not with the intention of unduly limiting the same.

#### EXAMPLE I

This example shows the effect of the addition of fluoride ions to the alumina.

These catalysts were prepared by adding ammonium hydroxide to aluminum chloride hexahydrate. The resultant alumina was washed very thoroughly in order to reduce the chloride content of the alumina to below 0.1% by weight on a dry basis. This washing entailed six separate washes with large amounts of water containing a small amount of ammonium hydroxide and finally an additional wash with water. In one catalyst preparation (designated as catalyst No. 1 in the following table) hydrogen sulfide at room temperature was bubbled through an aqueous solution of chloroplatinic acid and the resultant solution was added to the alumina in an amount to produce a final catalyst containing 0.1% by weight of platinum on a dry basis. The composite was then dried for 17 hours at 572° F. and then reduced with hydrogen at 932° F. for 3 hours.

A second catalyst was prepared in substantially the same manner as described for catalyst No. 1, except that hydrogen fluoride was intimately mixed with the alumina before the chloroplatinic acid-hydrogen sulfide solution was added thereto. The hydrogen fluoride was added as a 4.8% aqueous solution and was added in an amount to produce a final catalyst containing 1.5% by weight of fluorine.

These catalysts were used for the reforming of a Pennsylvania straight run naphtha having a boiling range of from 226° to 350° F. and an A. S. T. M. motor method octane number of 41.8, at a temperature of about 874° F., pressure of 500 pounds per square inch and a weight hourly space velocity of about 2. The liquid volume yield and the A. S. T. M. motor method octane number of the products are indicated in the following table:

Table 1

| No.    | Catalyst                               | Liquid Volume Yield per cent of Charge | Octane Number |
|--------|----------------------------------------|----------------------------------------|---------------|
| 1..... | No Fluorine in Catalyst.....           | 96                                     | 59.8          |
| 2..... | Catalyst Containing 1.5% Fluorine..... | 82.5                                   | 78.8          |

It will be noted that the catalyst containing fluorine yielded a reformate of 19 octane numbers higher than the catalyst containing no fluorine.

## EXAMPLE II

This example shows the effect of the addition of different amounts of fluorine to the catalyst. Catalysts No. 3 and No. 4 correspond to Catalyst No. 2 of Example I. Catalysts No. 5 and No. 6 were prepared in substantially the same manner as catalysts No. 3 and No. 4 except that the HF solution was added in an amount to produce a final catalyst containing fluorine in amounts of 3% for catalyst No. 5 and 6% for catalyst No. 6.

These catalysts were utilized for the reforming of the same gasoline described in Example I and under the same conditions of operation except that the temperature was varied as shown in the following table:

Table 2

| No.   | Catalyst          | Reforming Temp., °F. | Reformate Yield Wt. Percent of Charge | Exit Gas Wt. Percent of Charge | Octane No. |
|-------|-------------------|----------------------|---------------------------------------|--------------------------------|------------|
| 3.... | 1.5% Fluorine.... | 824                  | 95.9                                  | 3.6                            | 65.7       |
| 4.... | 1.5% Fluorine.... | 874                  | 83.2                                  | 6.9                            | 78.8       |
| 5.... | 3% Fluorine....   | 824                  | 85                                    | 4.9                            | 77.4       |
| 6.... | 6% Fluorine....   | 755                  | 77.6                                  | 4.5                            | 72.4       |

It will be noted from the above data that the temperature and fluoride concentration, at a constant space velocity, must be correlated in order to obtain the desired results. Referring to the run with catalyst No. 3, it will be noted that the temperature is too low because the octane number of the product was only 65.7. However, when the temperature was raised to 874° F., the octane number was increased to 78.8. Using the lower temperature (824° F.) with catalyst No. 5, satisfactory results were obtained. However, even lowering the temperature with catalyst No. 6 containing 6% fluorine, the octane number decreased. Therefore, the maximum fluorine content of the catalyst should not exceed about 3%.

## EXAMPLE III

This example shows the effect of chlorine content of the catalyst.

Catalysts No. 7, No. 8 and No. 9 comprised 0.1% platinum-alumina. The washing procedures were controlled to retain 0.5, 1.5 and 3.5% chlorine in the final catalyst.

These catalysts were used for the reforming of a Pennsylvania straight run naphtha having an initial boiling point of 219° F., an end boiling point of 339° F. and an A. S. T. M. motor method octane number of 41.2. These tests were conducted at a temperature of about 872° F., a pressure of about 500 pounds per square inch and a space velocity of about 2. The results of these tests are shown in the following table:

Table 3

| No.    | Catalyst           | Liquid Volume Yield Wt. Per-Cent of Charge | Octane Number |
|--------|--------------------|--------------------------------------------|---------------|
| 7..... | 0.5% Chlorine..... | 92.3                                       | 64.2          |
| 8..... | 1.5% Chlorine..... | 89.5                                       | 74.6          |
| 9..... | 3.5% Chlorine..... | 93.4                                       | 76            |

It will be noted that the catalyst containing 0.5% chlorine produced a reformate of 64.2 octane number. Therefore, the chloride content of the catalyst preferably is not below about 0.5% and certainly not below about 0.2%. Catalysts No. 8 and No. 9 containing higher concentrations of chlorine produced higher octane number prod-

ucts. However, the chlorine content should not be increased above about 8% and preferably not above about 5% because the catalyst will produce excessive hydro-cracking and result in an excess of gas formation.

## EXAMPLE IV

This example shows the beneficial effects obtained in preparing the catalyst by the use of hydrogen sulfide in the manner hereinbefore set forth. Catalyst No. 10 and No. 11 were prepared in substantially the same manner except that in catalyst No. 11 the mixture of alumina and chloroplatinic acid was heated to 140° F. and hydrogen sulfide was bubbled through the mixture for 15 minutes with constant stirring. The results of these tests are indicated in the following table:

Table 4

| No.     | Catalyst                  | Liquid Volume Yield Weight Percent of Charge | Octane Number |
|---------|---------------------------|----------------------------------------------|---------------|
| 10..... | Without Hydrogen Sulfide. | 96.2                                         | 69.3          |
| 11..... | With Hydrogen Sulfide.    | 89.7                                         | 78.4          |

It will be noted that the catalyst prepared by the addition of hydrogen sulfide gave a higher octane number product than the catalyst prepared in the absence of hydrogen sulfide.

## EXAMPLE V

This example shows the improved results obtained by adding chloroplatinic acid to wet alumina gel as compared to adding chloroplatinic acid to alumina which had been dried and formed into pills.

Catalyst No. 12 was prepared in substantially the same manner as hereinbefore set forth, while catalyst No. 13 was prepared by adding chloroplatinic acid to alumina pills which previously had been dried.

These catalysts were used for the reforming of a Mid-Continent straight run naphtha having an initial boiling point of 217° F., an end boiling point of 392° F. and an A. S. T. M. motor method octane number of 38.9. The reforming was effected at a temperature of 752° F., pressure of 200 pounds per square inch and a space velocity of 1. The results are shown in the following table:

Table 5

| No.     | Catalyst                              | Liquid Volume Yield | Octane Number |
|---------|---------------------------------------|---------------------|---------------|
| 12..... | Platinum added to wet alumina slurry. | 92.8                | 68.2          |
| 13..... | Platinum added to dry alumina pills.  | 97.6                | 50            |

It will be noted that the catalyst prepared by the addition of chloroplatinic acid to wet alumina slurry produced a considerably higher octane number product under the same conditions of operation.

## EXAMPLE VI

This example shows the effect of temperature of hydrogen sulfide addition in catalysts prepared by adding the hydrogen sulfide to the chloroplatinic acid solution and then adding this mixture to the wet alumina slurry. In catalyst No.

## 11

14 the hydrogen sulfide was added at room temperature, whereas in catalyst No. 15 the hydrogen sulfide was passed through a solution of chloroplatinic acid at 176° F. These catalysts were tested in the reforming of a Pennsylvania straight run naphtha having an initial boiling point of 226° F., an end boiling point of 350° F. and an A. S. T. M. motor method octane number of 41.8. The results of these tests are shown in the following table:

Table 6

| No.     | Catalyst                                    | Liquid Volume Yield | Octane Number |
|---------|---------------------------------------------|---------------------|---------------|
| 14..... | Hydrogen sulfide added at room temperature. | 96.7                | 60.1          |
| 15..... | Hydrogen sulfide added at 176° F...         | 97.7                | 58.4          |

It will be noted that the catalysts prepared by adding the hydrogen sulfide at room temperature produced a somewhat higher octane number product than the catalyst prepared by adding the hydrogen sulfide at an elevated temperature.

## EXAMPLE VII

This example shows the effect of temperature of hydrogen sulfide addition in catalysts prepared by commingling the chloroplatinic acid with the alumina gel and then introducing the hydrogen sulfide.

Catalyst No. 16 was prepared by adding the hydrogen sulfide at room temperature, while catalyst No. 17 was prepared by adding the hydrogen sulfide at a temperature of 158° F. The results are shown in the following table:

Table 7

| No.     | Catalyst                                    | Liquid Volume Yield | Octane Number |
|---------|---------------------------------------------|---------------------|---------------|
| 16..... | Hydrogen sulfide added at room temperature. | 94.4                | 63.8          |
| 17..... | Hydrogen sulfide added at 158° F...         | 95.6                | 62.8          |

It will be noted that the results are fairly comparable in these tests and that the effect of temperature of hydrogen sulfide treatment is not substantial in catalysts prepared by adding hydrogen sulfide to the chloroplatinic acid-alumina gel mixture.

## EXAMPLE VIII

In view of the very low concentrations of platinum found to be effective in catalyzing the reforming operation, the questions naturally arise as to whether such small amounts of platinum are actually of any effect and whether the platinum can not be omitted and the same results obtained. In order to definitely show that improved results are obtained through the use of these small amounts of platinum, two catalysts were prepared in substantially the same manner except that one catalyst comprised 0.1% by weight of platinum composited with alumina, and the other catalyst comprised alumina but contained no platinum.

In a reforming operation, a Pennsylvania straight run naphtha having a boiling range of from 226° F. to 350° F. and an A. S. T. M. motor method octane number of 41.8 was subjected to conversion in the presence of the platinum-containing catalyst and in the presence of the catalyst containing no platinum at a temperature of

## 12

about 872° F., a pressure of 500 pounds per square inch and a weight hourly space velocity of about 2. The liquid volume yield and the A. S. T. M. motor method octane number of the products are indicated in the following table:

Table 8

| 10 | No.     | Catalyst                   | Liquid Volume Yield Percent of Charge | Octane Number |
|----|---------|----------------------------|---------------------------------------|---------------|
| 15 | 18..... | 0.1% platinum alumina..... | 81.6                                  | 80            |
|    | 19..... | alumina.....               | 99                                    | 50.6          |

It will be noted that the catalyst containing no platinum yielded a product of 50.6 octane number, whereas the platinum containing catalyst yielded a product of 80 octane number. It is readily apparent that the 0.1% by weight of platinum exerts a definite catalytic effect.

I claim as my invention:

1. A process for reforming a gasoline fraction which comprises subjecting said fraction to contact at reforming conditions with a catalyst comprising alumina, platinum and combined halogen.

2. The process of claim 1 further characterized in that said halogen is in an amount of from about 0.1% to about 8% by weight of said catalyst.

3. The process of claim 2 further characterized in that said halogen comprises fluorine in an amount of from about 0.1% to about 3% by weight of said catalyst.

4. The process of claim 1 further characterized in that said halogen comprises chlorine in an amount of from about 0.2% to about 8% by weight of said catalyst.

5. The process of claim 1 further characterized in that said platinum is in an amount of from about 0.01% to about 1% by weight of said catalyst.

6. A process for reforming a saturated gasoline fraction which comprises subjecting said fraction to contact at reforming conditions with a catalyst comprising alumina, platinum in an amount of from about 0.01% to about 1% by weight of said catalyst, and combined fluorine in an amount of from about 0.1% to about 3% by weight of said catalyst.

7. A process for reforming a saturated gasoline fraction which comprises subjecting said fraction to contact at reforming conditions with a catalyst comprising alumina, platinum in an amount of from about 0.01% to about 1% by weight of said catalyst, and combined chlorine in an amount of from about 0.2% to about 8% by weight of said catalyst.

8. A process for reforming a straight run gasoline fraction which comprises subjecting said fraction to contact at a temperature of from about 600° to about 1000° F., a pressure of from about 50 to about 1000 pounds per square inch and a weight hourly space velocity of from about 0.5 to 10, in the presence of from about 0.5 to about 10 mols of hydrogen per mol of hydrocarbon, with a catalyst comprising alumina, platinum in an amount of from about 0.01% to about 1% by weight of said catalyst, and combined fluorine in an amount of from about 0.1% to about 3% by weight of said catalyst.

9. A process for reforming a straight run gasoline fraction which comprises subjecting said fraction to contact at a temperature of from about 600° to about 1000° F., a pressure of from

13

about 50 to about 1000 pounds per square inch and a weight hourly space velocity of from about 0.5 to 10, in the presence of from about 0.5 to about 10 mols of hydrogen per mol of hydrocarbon, with a catalyst comprising alumina, platinum in an amount of from about 0.1% to about 1% by weight of said catalyst, and combined chlorine in an amount of from about 0.5% to about 5% by weight of said catalyst.

10. A process for reforming a gasoline fraction which comprises subjecting said fraction to contact at reforming conditions with a catalyst prepared by forming a mixture of alumina and halogen ions, the halogen ions being in an amount of from about 0.1% to about 8% by weight of said alumina on a dry basis, thereafter commingling platinum with the mixture, and subsequently heating the composite.

11. A process for reforming a gasoline fraction which comprises subjecting said fraction to contact at reforming conditions with a catalyst prepared by forming alumina from an aluminum salt, commingling halogen ions therewith in an amount of from about 0.1% to about 8% by weight of said alumina, thereafter commingling with the mixture a platinum solution in an amount to form a final catalyst containing from about 0.01% to about 1% by weight of platinum, and heating the composite at a temperature of from about 800° to about 1200° F.

12. A process for reforming a gasoline fraction which comprises subjecting said fraction to contact at reforming conditions with a catalyst prepared by forming alumina from aluminum chloride, washing to remove chloride ions to below about 0.1% by weight of said alumina, adding fluoride ions in an amount of from about 0.1% to about 3% by weight of said alumina, separately commingling hydrogen sulfide at substantially room temperature with a chloroplatinic acid solution, commingling the resultant solution at substantially room temperature with said alumina containing fluorine, and thereafter heating the resultant composite at a temperature of from about 800° to about 1200° F.

13. A process for reforming a gasoline fraction which comprises subjecting said fraction to contact at reforming conditions with a catalyst prepared by forming alumina from aluminum chloride, washing to remove chloride ions to below about 0.1% by weight of said alumina, adding chloride ions in an amount of from about 0.5% to about 5% by weight of said alumina, separately commingling hydrogen sulfide at substantially room temperature with a chloroplatinic acid solution, commingling the resultant solution at substantially room temperature with said alumina containing chlorine, and thereafter heating the resultant composite at a temperature of from about 800° to about 1200° F.

14. A process for reforming a gasoline fraction which comprises subjecting said fraction to contact at reforming conditions with a catalyst prepared by forming alumina from aluminum chloride, washing to remove chloride ions to below about 0.1% by weight of said alumina, commingling fluoride ions in an amount of from about 0.1% to about 3% by weight of said alumina, adding chloroplatinic acid solution in an amount to form a final catalyst containing from about 0.1% to about 1% by weight of platinum, adding hydrogen sulfide to the resultant mixture, and thereafter heating the same at a temperature of from about 800° to about 1200° F.

15. A process for reforming a gasoline fraction

14

which comprises subjecting said fraction to contact at reforming conditions with a catalyst prepared by forming alumina from aluminum chloride, washing to remove chloride ions to below about 0.1% by weight of said alumina, commingling chloride ions in an amount of from about 0.5% to about 5% by weight of said alumina, adding chloroplatinic acid solution in an amount to form a final catalyst containing from about 0.1% to about 1% by weight of platinum, adding hydrogen sulfide to the resultant mixture, and thereafter heating the same at a temperature of from about 800° to 1200° F.

16. A process for reforming a gasoline fraction which comprises subjecting said fraction to contact at reforming conditions with a catalyst prepared by forming alumina from aluminum chloride, washing with water containing ammonium hydroxide to remove chloride ions to below about 0.1% by weight of said alumina, adding a dilute aqueous solution of hydrogen fluoride to said alumina in an amount to form a final catalyst containing from about 0.1% to about 3% by weight of fluoride ions based on said alumina, separately commingling hydrogen sulfide with a chloroplatinic acid solution in an amount to form a final catalyst containing from about 0.01% to about 1% by weight of platinum, commingling the resultant solution with said alumina containing fluoride ions, and thereafter heating the resultant composite at a temperature of from about 800° to about 1200° F.

17. A process for reforming a gasoline fraction which comprises subjecting said fraction to contact at reforming conditions with a catalyst prepared by forming alumina from aluminum chloride, washing with water containing ammonium hydroxide to remove chloride ions to below about 0.1% by weight of said alumina, adding a dilute aqueous solution of hydrogen chloride to said alumina in an amount to form a final catalyst containing from about 0.2% to about 8% by weight of chloride ions based on said alumina, separately commingling hydrogen sulfide with a chloroplatinic acid solution in an amount to form a final catalyst containing from about 0.01% to about 1% by weight of platinum, commingling the resultant solution with said alumina containing chloride ions, and thereafter heating the resultant composite at a temperature of from about 800° to about 1200° F.

18. A process for reforming a straight run gasoline fraction which comprises subjecting said fraction to contact at a temperature of from about 600° to about 1000° F., a pressure of from about 50 to about 1000 pounds per square inch, and a weight hourly space velocity of from about 0.5 to about 10, in the presence of from about 0.5 to about 10 mols of hydrogen per mol of hydrocarbon, with a catalyst prepared by forming alumina from aluminum chloride, washing to remove chloride ions to below about 0.1% by weight of said alumina, adding a dilute aqueous solution of hydrogen fluoride to said alumina in an amount to form a final catalyst containing from about 0.1% to about 3% by weight of fluoride ions based on said alumina, separately commingling hydrogen sulfide with a chloroplatinic acid solution in an amount to form a final catalyst containing from about 0.01% to about 1% by weight of platinum, commingling the resultant solution with said alumina containing fluoride ions, and thereafter heating the resultant composite at a temperature of from about 800° to about 1200° F.

75 temperature of from about 800° to about 1200° F.

19. A process for reforming a gasoline fraction which comprises subjecting said fraction to contact at reforming conditions with a catalyst comprising a major proportion of alumina, from about 0.01% to about 1% by weight of platinum, and from about 0.1% to about 8% by weight of combined halogen.

VLADIMIR HAENSEL.

5

## REFERENCES CITED

The following references are of record in the file of this patent:

## UNITED STATES PATENTS

| Number    | Name                 | Date          |
|-----------|----------------------|---------------|
| 2,184,235 | Groll et al. -----   | Dec. 19, 1939 |
| 2,411,726 | Holroyd et al. ----- | Nov. 26, 1946 |